

Oct. 4, 1932.

B. E. EISEN HOUR

1,880,923

COMPENSATED TUNING FORK

Filed Sept. 4, 1930



*Inventor:  
Bert E. Eisenhour,  
By: Wallace R. Lane Atty.*

## UNITED STATES PATENT OFFICE

BERT E. EISENHOOR, OF AURORA, ILLINOIS, ASSIGNOR OF ONE-HALF TO GEORGE FABYAN, OF GENEVA, ILLINOIS

## COMPENSATED TUNING FORK

Application filed September 4, 1930. Serial No. 479,698.

The present invention relates to tuning forks, and is directed to compensating tuning forks so that the pitch or vibration frequencies thereof will remain constant irrespective of the temperature or change of temperature of the tuning forks, or can be made any value within the limits of the elastic coefficients of the material used.

In a tuning fork, the pitch or vibration frequency thereof, changes with a change of length and elasticity of the material. An increase of length will cause a decrease or lowering of the pitch or vibration frequency. A decrease of length will raise or increase the pitch or vibration frequency. A decrease of elasticity will cause a lowering or decrease in pitch or vibration frequency, and an increase of elasticity will raise or increase the pitch or vibration frequency.

Hence, when a fork is heated or rises in temperature, the fork expands and its elasticity is decreased. Both of these factors produce a drop in pitch. When the fork is cooled or lowered in temperature, the fork contracts and its elasticity increases. Both these factors raise the pitch. These characteristics are peculiar to most materials used for making tuning forks.

Various metals known in the trade as stoic metals, such as elinvar, (invar, and other iron and nickel alloys) have the property of increasing and decreasing their elasticity upon increase and decrease in temperature respectively. This characteristic of stoic metals may be made to counteract the characteristics pointed out above as peculiar to the materials usually used for making tuning forks.

An object of the present invention is to provide a novel tuning fork composed of different metals having opposite temperature co-efficient values which will balance and maintain the tuning fork at a constant pitch or vibration frequency irrespective of the temperature or change of temperature of the fork. Such metals may be combined in the proportions inversely to such values. As for example, when steel is used as one component and elinvar as the other, and if the temperature co-efficient values of the steel be about

ten times that of the opposite temperature co-efficient value of the elinvar, then the resulting fork may be composed in the proportions of about ten parts of elinvar to one part of steel.

Other objects, advantages, capabilities and features are comprehended by the invention as will later appear and as are inherently possessed thereby.

Referring to the drawing:

Figs. 1, 2 and 3 are perspective views of alternative forms of tuning forks constructed in accordance with the invention.

Referring more in detail to the drawing, the particular embodiments selected to illustrate the invention, are shown in the form of laminated forks.

In Fig. 1, the fork comprises leg laminae 1, 2, 3 and 4 of which laminae 1 and 2 are connected by the usual form of cross-head 5 carrying a stem 6.

In Fig. 2 the fork comprises leg laminae 1<sup>a</sup>, 2<sup>a</sup>, 3<sup>a</sup>, 3<sup>b</sup>, 4<sup>a</sup>, and 4<sup>b</sup>, the cross-head also comprising cross head laminae 5<sup>a</sup>, 5<sup>b</sup> and 5<sup>c</sup>. The stem 6<sup>a</sup> is connected to the lamina 5<sup>c</sup>.

In Fig. 3 the fork comprises leg laminae 1<sup>c</sup>, 1<sup>d</sup>, 2<sup>c</sup>, 2<sup>d</sup>, 3<sup>c</sup> and 4<sup>c</sup> cross-head laminae 5<sup>d</sup>, 5<sup>e</sup> and 5<sup>f</sup>. The stem 6<sup>c</sup> is connected to the cross-head.

In each of these, the laminae 3, 4, 3<sup>a</sup>, 3<sup>b</sup>, 4<sup>a</sup>, 4<sup>b</sup>, 3<sup>c</sup> and 4<sup>c</sup>, may be of any usual material used for making tuning forks, such as steel or other similar material, while the other laminae 1, 2, 1<sup>a</sup>, 2<sup>a</sup>, 1<sup>c</sup>, 2<sup>c</sup>, 1<sup>d</sup> and 2<sup>d</sup> are of material having a temperature co-efficient value opposite to that of the steel and the like, such as invar, elinvar or like metals or alloys. The former laminae may be secured to the edges of the fork (as in Fig. 1), or the sides of the fork (as in Fig. 2), or intermediately of the fork (as in Fig. 3), in any suitable manner, as by soldering, welding, brazing, rivets, screws, and the like.

By regulating or adjusting the proportions and similar physical properties of the different metals, it is possible to control the frequency or period of vibration of the fork when subjected to changes in temperature. To secure such control, it is necessary that the two different metals or alloys have oppo-

55

60

65

70

75

80

85

90

95

100

site values for the temperature coefficient of elasticity.

For the purpose of giving an example, it will be assumed that the laminæ 3 and 4 (Fig. 1) 3<sup>a</sup>, 3<sup>b</sup>, 4<sup>a</sup>, and 4<sup>b</sup> (Fig. 2) and 3<sup>c</sup> and 4<sup>c</sup> (Fig. 3) are of steel having a temperature coefficient of elasticity of  $62.2 \times 10^{-6}$ . This is negative in value for the reason that with increase in temperature, the elasticity will decrease and hence the frequency or pitch will be lowered in a tuning fork. The other laminæ must be opposite or positive in value and the temperature coefficient of elasticity thereof equal to that of the steel, so that an increase in temperature will effect an increase in elasticity and hence increase the frequency or pitch of the fork. With these two metals firmly connected together, and with the different laminæ tuned to approximately the same frequency before assembling, the resultant assembly will have the same frequency and the system is balanced without stresses and strains.

If now the system be heated, the laminæ having the negative value will tend to decrease the pitch and the laminæ having the positive value will tend to increase the pitch, and since these opposing forces are equal, there is no change and the entire system remains with a constant or fixed pitch or vibration frequency.

In a specific case, a tuning fork component of elinvar of given dimensions was made for a frequency of 512 D. V. and measured over a temperature range of 32° to 212° F. and the temperature coefficient of frequency found to be  $5.17 \times 10^{-6}$  positive. A similar component of steel with a little more than one tenth the thickness of the elinvar component was made for the same frequency and likewise measured for its temperature coefficient of frequency which was found to be  $62.2 \times 10^{-6}$  negative. These two components were united and the resultant fork tested with the result that its temperature coefficient of frequency was  $5.11 \times 10^{-6}$  negative. This was then adjusted or regulated by removing some material from the steel component to bring down the temperature coefficient of frequency to as low a value as desired or possible. A fork assembly of this invention was brought to  $0.225 \times 10^{-6}$  negative and was for practical purposes, substantially permanent or perfect. The ultimate, with measuring instruments sufficiently sensitive, would be to obtain a value of zero for the temperature coefficient of frequency.

The temperature coefficient of frequency of a tuning fork is equal to the temperature coefficient of elasticity minus the temperature coefficient of expansion, divided by the factor 2, and is expressed by the formula:

$$A = \frac{y-z}{2}$$

65

Where A is the temperature coefficient of frequency of the fork, y is the temperature coefficient of the modulus of elasticity, and z is the temperature coefficient of expansion.

The value y is negative and the value z is positive for steel, so that the two effects are additive, both causing the temperature coefficient of the tuning fork to be negative, that is, a rise in temperature causes a decrease in frequency. Some alloys having nickel and iron as their principal components, such as invar and elinvar, have a positive temperature coefficient of elasticity and a positive temperature coefficient of expansion, so that these effects are subtractive. By combining nickel-iron and carbon-steel in correct proportions, the positive temperature coefficient of elasticity of the nickel-iron counteracts the effect of the three other temperature coefficients.

The fork of the present invention, is composed of about 1/10 part of steel having a temperature coefficient of elasticity of  $-354 \times 10^{-6}$  and a temperature coefficient of expansion of  $+12 \times 10^{-6}$ , and about 9/10 parts of invar or elinvar having a temperature coefficient of elasticity of  $+50 \times 10^{-6}$  and a temperature coefficient of expansion of  $+6 \times 10^{-6}$ . The temperature coefficient of frequency is the summation of these. Such is represented by the equation:

$$\frac{1/10 \times (-354) \times 10^{-6}}{2} \frac{1/10 \times 12 \times 10^{-6}}{2} + \frac{9/10 \times 50 \times 10^{-6}}{2} \frac{9/10 \times 6 \times 10^{-6}}{2} = \frac{3 \times 10^{-6}}{2} = +0.0000015$$

105

This last value is practically a zero quantity, thus showing that the frequency of the fork is practically constant for any range of temperature.

When the proportions are 10.7318% of steel and 89.2682% of invar or elinvar, this value becomes  $-0.000,000,000,03$  and when the proportions are 10.7317% of steel and 89.2683% of invar or elinvar, this value becomes  $+0.000,000,000,015$ . The absolute zero value would occur when the steel is between 10.7317% and 10.7318% and the invar or elinvar is between 89.2682% and 89.2683%.

The physical properties and characteristics of elinvar as given by its manufacturer, are as follows:

Specific gravity 8.14 to 8.16.

Modulus of elasticity of torsion at 15° C. from 670 to 7100 kg/m/m<sup>2</sup>.

Modulus of elasticity of traction at 15° C. from 18,000 to 19,000 kg/m/m<sup>2</sup>.

Temperature coefficient of modulus of elasticity (torsion and traction)  $\pm 50 \times 10^{-6}$ .

Temperature coefficient of temperature of dilation at 15° C. from  $6 \times 10^{-6}$  to  $6.5 \times 10^{-6}$ .

130

While I have herein described, and upon the drawing shown a few illustrative embodiments of the invention, it is to be understood that the latter is not limited thereto but may 5 comprehend other constructions, details, arrangements of parts, and features without departing from the spirit thereof.

Having thus disclosed the invention, I claim:

- 10 1. A tuning fork composed of laminations of metals having opposite values for the temperature coefficients of elasticity of said metals for maintaining the vibration frequency of the fork constant under changes 15 of temperature of the fork.
  - 15 2. A tuning fork composed of laminations of metals having positive and negative temperature coefficients of elasticity of the metals for maintaining the vibration frequency of 20 the fork constant under changes of tempera- ture of the fork.
  - 25 3. A tuning fork composed of laminations of metals of which one metal has the prop- erty of varying the vibration frequency of the fork directly with the change in tempera- ture of the fork, and another metal has the property of varying the vibration frequency of the fork inversely with the change in tempera- ture of the fork, for maintaining the 30 vibration frequency of the fork constant under changes of temperature of the fork.
  - 35 4. A tuning fork composed of laminations of metals of which one metal has a tempera- ture coefficient of elasticity of a value equal to and opposite to the values of the tempera- ture coefficient of elasticity of the other metal and of the temperature coefficients of expansion of both metals.
  - 40 5. A tuning fork composed of laminations of different metals having opposite values of temperature coefficients of elasticity for giving to the fork a given vibration frequency which will remain constant under changes of temperature of the fork.
  - 45 6. A tuning fork composed of laminations of combined metals in the proportions of the coefficients of elasticity values thereof, said values being opposite.
  - 50 7. A tuning fork comprising laminations of different metals having opposite tempera- ture coefficients of elasticity.
  - 55 8. A tuning fork comprising laminations of different metals having opposite tempera- ture coefficients of elasticity and in the pro- portions of the values of said coefficients.
  - 60 9. A tuning fork composed of steel and elinvar laminations.
  - 65 10. A tuning fork composed of laminations in the proportions of about ten parts of elin- var and one part of steel.
- In witness whereof, I hereunto subscribe my name to this specification.
- BERT E. EISENHOUR.

**CERTIFICATE OF CORRECTION.**

Patent No. 1,880,923.

**October 4, 1932.**

**BERT E. EISENHOUR.**

It is hereby certified that error appears in the printed specification of the above numbered patent requiring correction as follows: Page 2, line 124, for 670" read "6700"; and that the said Letters Patent should be read with this correction therein that the same may conform to the record of the case in the Patent Office.

Signed and sealed this 29th day of November, A. D. 1932.

(Seal)

**M. J. Moore,  
Acting Commissioner of Patents.**